# EUROPEAN PATENT SPECIFICATION

(11) **EP 0 375 179 B1**
(45) Date of publication and mention of the grant of the patent: **25.05.1994**
(21) Application number: 89312444.6
(22) Date of filing: 29.11.1989
(51) Int. Cl.: C25D 3/38, C25D 5/30, C25D 5/28

(54) **Copper plating process for difficult to plate metals**
Kupfer-Plattierungsverfahren für Metalle, die schwer zu plattieren sind
Procédé de placage du cuivre sur des métaux difficiles à plaquer

(30) Priority: 21.12.1988 US 289993
(43) Date of publication of application: 27.06.1990
(73) Proprietor: International Business Machines Corporation, Armonk, N.Y. 10504 (US)
(72) Inventor: Mahmoud, Issa Said, Austin Texas 78750 (US)
(74) Representative: Burt, Roger James, Dr.

(56) References cited:
- METALOBERFLÄCHE, vol. 33, no. 1, 1979, pages 9-16; M.F.M. EL GHANDOUR et al.: "Einfluss von Harnstoff und anderen Zusätzen, sowie der Herstellungsbedingungen auf die elektrolytische Abscheidung von Kupfer aus Kupfersulfatbädern"
- CHEMICAL ABSTRACTS, vol. 96, no. 24, 14th June 1982, page 531, abstract no. 207474k, Columbus, Ohio, US; & SU-A-901 363 (V.M. GOLIKOV et al.) 30-01-1982

## Description

The present invention relates to an electroplating bath composition suitable for electroplating extremely electropositive metals such as aluminium and tungsten.

Strongly electropositive metals such as aluminium and tungsten are quite difficult to electroplate. Such metals have a strong affinity for atmospheric oxygen. This characteristic creates an ever present compacted oxide layer at the metal surface. Such a layer forms within seconds after a fresh surface of these metals is exposed to oxygen. The oxide layer renders plating these metals very difficult; and if plating occurs, in many cases, the adhesion is quite poor.

Conventional techniques for plating such metals include extensive surface pre-treatment. In the case of tungsten, parts to be plated are often transferred from tank to tank while under electrical bias, thereby creating a safety hazard due to the possibility of electrical shock. Additionally, conventional plating processes for these metals generate significant amounts of harsh waste, such as hydrofluoric acid.

Thus, a better process and plating bath chemistry is desirable for plating these difficult to plate metals. U.S. Patent 3,769,179 to Durose et al, U.S. Patent 4,242,181 to Malak and 3,923,613 to Immel, exemplify the prior art of copper plating; the first two particularly, as applied to the printed circuit manufacturing industry.

The present invention provides a process including a bath formulation for depositing copper on difficult to plate metals such as aluminium and tungsten. The bath formulation of the present invention is an acid copper bath and includes additives for specific purposes.

The process of the present invention requires no surface preparation or etching prior to plating, thereby reducing the amount of chemical waste attendant to the process. Further, the present invention provides for oxide removal from difficult to plate metals in the plating tank so that there is minimal opportunity for new oxide to form on clean surfaces, thereby enabling the establishment of excellent metallic bonds between the electrodeposited copper and base metal.

The inventive process provides higher yields, better adhesion while minimizing the cost associated with waste treatment.

The preferred aqueous plating solution contains sulphuric acid, 0.5-0.75 moles per litre; hydrated copper sulphate, 0.3-0.5 moles per litre; urea, 1-2 grammes per litre; a wetting agent, 1-2 millilitres per litre; sulphonic acid, 1-2 grammes per litre; and deionized water, 800-1000 millilitres.

More particularly, the preferred solution composition includes 0.5 mol. hydrated copper sulphate, 0.4 mol. sulphuric acid, 1 gramme urea, 1 gramme Beta-phenylethyltosylate (an ester of a sulphonic acid) and sufficient water to make one litre of solution. Preparation of the bath is preferably carried out as follows. About 700 millilitres of deionised or distilled water is measured into a 2000 ml beaker, to which is added the above bath constituents in the order listed with continuous agitation. Subsequently enough water is added to make one litre of solution which is then filtered to remove any undissolved reagents.

Urea is included for its properties as a levelling agent. Sulphonic acid is used for its brightening properties. Sulphonic acids of the ester type, particularly of the tosyl and mesyl types, are well suited for use in the present plating bath solution. Suitable wetting agents include cationic surfactants such as sodium lauryl sulphate.

The bath is prepared by adding all of the chemicals in the order listed to the deionized water. The solution is mixed and filtered if need be to remove any undissolved particles. Metals to be plated are first cleaned to remove soil, dirt and other surface contaminants, then rinsed in deionized water. The metals are then placed in the plating tank containing the prepared bath.

Preferably, the parts remain in the plating solution for 2 to 3 minutes before a negative bias is applied to commence electroplating of copper. However, it has been noted that in some difficult cases, if the parts are given a positive bias for 30 to 60 seconds before the negative bias is applied, particularly stubborn, naturally grown oxide layers may be removed.

Normal plating process parameters include a bath temperature in the range of 20-30 degrees Celsius, at a current density of 108-216 amperes per square metre (10-20 amperes per square foot) With continuous, strong agitation. The duration of the plating step is variable, depending on the desired copper thickness.

The sulphuric acid concentration in the plating bath is sufficient for removing the oxide layers during the 2-3 minute soak before introduction of current. No extensive surface preparation or etching is required before plating, thereby reducing the number of steps and the amount of chemical waste generated and the cost attendant thereto.

The following examples are illustrative of the various aspects of the invention.

### Example 1

Aluminium and tungsten workpieces were cleaned in a mild alkaline cleaner and then plated in the following solution:
Sulphuric acid, 75 grammes/litre
Hydrated Copper sulphate, 72 grammes/litre
Urea (levelling agent), 1 gramme/litre
Sulphonic acid (brightener), 1 gramme/litre
Sodium lauryl sulphate surfactant, 1 gramme/litre
Deionized water, 1 litre
The workpieces were immersed in this solution for 2-3 minutes prior to biasing. Plating was carried out at room temperature and at 108 amperes per square metre (10 amperes per square foot) for 20 minutes. The copper deposits were smooth and free of defects such as skip plating. Testing for adhesion strength by both cross-cut and quench method showed no adhesion failures.

### Example 2

Another example of this invention was carried out in a similar manner as Example 1, except the amount of sulphuric acid was reduced to 50 grammes/litre. Again the quality and adhesion of the copper deposit were similar to Example 1.

### Example 3

Another experiment was carried out as in Examples 1 and 2, except that the concentration of sulphuric acid was further reduced to 30 grammes/litre. Subsequent adhesion testing showed failures at more than 25% of the tested areas.

### Example 4

In another example the conditions were as in Example 1 except that the amount of hydrated copper sulphate was 50 grammes/litre. The electrodeposits were smooth, free of skip plating and had excellent adhesion.

### Example 5

Coupons of tungsten which showed slight blue colour (tungsten oxide) were cleaned and then plated as in Example 1. Subsequent adhesion testing showed poor adhesion. However, when the coupons were first positively biased for 1 minute, then plated in the negative bias, the plated coupons showed good adhesion.

## Claims

1. An acid copper plating bath for electropositive metals consisting essentially of:
0.5 to 0.75 mols per litre sulphuric acid;
0.3 to 0.5 mols per litre hydrated copper sulphate;
1 to 2 grams per litre, urea;
1 to 2 millilitres per litre, wetting agent;
1 to 2 grams per litre, tosyl or mesyl sulphonic acid ester as a brightening agent; and
800 - 1000 millilitres deionized water.

2. An aqueous acid copper plating bath for electropositive metals comprising:
sulphuric acid, 30 to 50 grams/litre;
hydrated copper sulphate 75 to 125 grams/litre;
urea, 1 gram/litre;
tosyl or mesyl sulphonic acid ester, 1 gram/litre; and
wetting agent, 1 gram/litre.

3. A copper plating bath as claimed in claim 1 or claim 2 wherein the wetting agent is a cationic surfactant.

4. A copper plating bath as claimed in claim 3 wherein the cationic surfactant is sodium lauryl sulphate.

5. A copper plating bath as claimed in any of the preceding claims wherein the sulphonic acid ester is Beta-phenylethyltosylate.

6. A process for copper plating electropositive metals comprising the steps of:
preparing a bath containing
0.5 to 0.75 mols per litre sulphuric acid;
0.3 to 0.5 mols per litre hydrated copper sulphate;
1 to 2 grams per litre urea;
1 to 2 millilitres per litre sodium lauryl sulphate;
1 to 2 grammes per litre a tosyl or mesyl sulphonic acid ester; and
800 to 1000 millilitres deionized water;
soaking parts to be plated in the bath; and
electrodepositing copper from the bath at a temperature of about 20 to 30 degrees Celsius at a current density of 108 to 216 amperes per square metre (10 - 20 amperes per square foot), with continuous agitation.

7. The process of Claim 6 wherin the soaking step is 2 to 3 minutes in duration.

8. The process of Claim 6 wherein the soaking step lasts for 30 to 60 seconds under the influence of a positive bias.

9. The process of Claim 6 wherein the preparing step includes:
mixing of bath components in the order set forth in Claim 6, in deionized water; and
filtering the bath solution.

## Patentansprüche

1. Ein Säure-Kupferplattierungsbad für elektropositive Metalle, das sich im wesentlichen zusammensetzt aus:
0,5 bis 0,75 Mol/Liter Schwefelsäure;
0,3 bis 0,5 Mol/Liter hydriertem Kupfersulfat;
1 bis 2 Gramm/Liter Urea;
1 bis 2 ml/Liter Wässerungsmittel;
1 bis 2 Gramm/Liter Tosyl- oder Mesyl-Sulfonsäureester (als Aufhellungsmittel); und
800 bis 1000 ml deionisiertem Wasser.

2. Ein wässriges Säure-Kupferplattierungsbad für elektropositive Metalle, bestehend aus:
Schwefelsäure, 30 bis 50 Gramm/Liter;
hydriertem Kupfersulfat, 75 bis 125 Gramm/Liter;
Urea, 1 Gramm/Liter;
Tosyl- oder Mesyl-Sulfonsäureester, 1 Gramm/Liter; und
Wässerungsmittel, 1 Gramm/Liter.

3. Ein Kupferplattierungsbad gemäß Anspruch 1 oder Anspruch 2, bei dem das Wässerungsmittel ein kationisches Tensid ist.

4. Ein Kupferplattierungsbad gemäß Anspruch 3, bei dem das kationische Tensid Natriumlaurylsulfat ist.

5. Ein Kupferplattierungsbad gemäß allen vorherigen Ansprüchen, bei dem das Sulfonsäureester Beta-phenylethyltosylat ist.

6. Ein Verfahren zur Plattierung elektropositiver Metalle wie Kupfer, bestehend aus den Schritten:
Vorbereitung eines Bads, das folgendes enthält:
0,5 bis 0,75 Mol/Liter Schwefelsäure;
0,3 bis 0,5 Mol/Liter hydriertes Kupfersulfat;
1 bis 2 Gramm/Liter Urea;
1 bis 2 ml/Liter Natriumlaurylsulfat;
1 bis 2 Gramm/Liter Tosyl- oder Mesyl-Sulfonsäureester; und
800 bis 1000 ml deionisiertes Wasser.
Eintauchen der zu plattierenden Teile in das Bad; und
elektrolytische Beschichtung mit Kupfer im Bad bei einer Temperatur von ungefähr 20 bis 30°C und einer Stromdichte von 108 bis 216 Ampère/m² und bei kontinuierlichem Umrühren.

7. Das Verfahren aus Anspruch 6, wobei der Eintauchschritt 2 bis 3 Minuten dauert.

8. Das Verfahren aus Anspruch 6, wobei der Eintauchschritt unter dem Einfluß einer positiven Vorspannung 30 bis 60 Sekunden dauert.

9. Das Verfahren aus Anspruch 6, wobei der Vorbereitungsschritt folgendes umfaßt:
Mischen der Badbestandteile in der in Anspruch 6 aufgeführten Reihenfolge in deionisiertem Wasser; und
Filtern der Badlösung.

## Revendications

1. Bain de cuivrage acide pour métaux électropositifs, comprenant essentiellement :
0,5 à 0,75 moles par litre d'acide sulfurique;
0,3 à 0,5 moles par litre de sulfate de cuivre hydraté;
1 à 2 grammes par litre d'urée;
1 à 2 millilitres par litre d'un agent mouillant;
1 à 2 grammes par litre d'ester d'acide sulfonique tosyl ou mésyl, comme agent de blanchiment; et
800 à 1.000 millilitres d'eau déminéralisée.

2. Bain de cuivrage acide aqueux pour métaux électropositifs, comprenant :
30 à 50 grammes/litre d'acide sulfurique;
75 à 125 grammes/litre de sulfate de cuivre hydraté;
1 gramme/litre d'urée;
1 gramme/litre d'ester d'acide sulfonique tosyl ou mésyl; et
1 gramme/litre d'un agent mouillant.

3. Bain de cuivrage selon la revendication 1 ou 2, dans lequel l'agent mouillant est un agent de surface cationique.

4. Bain de cuivrage selon la revendication 3, dans lequel l'agent de surface cationique est du sulfate laurique de sodium.

5. Bain de cuivrage selon l'une quelconque des revendications précédentes, dans lequel l'ester d'acide sulfonique est du phényléthyltosylate-bêta.

6. Procédé pour le cuivrage des métaux électropositifs, comprenant les étapes consistant à :
préparer un bain contenant
0,5 à 0,75 moles par litre d'acide sulfurique;
0,3 à 0,5 moles par litre de sulfate de cuivre hydraté;
1 à 2 grammes par litre d'urée;
1 à 2 millilitres par litre d'un agent mouillant;
1 à 2 grammes par litre d'ester d'acide sulfonique tosyl ou mésyl, comme agent de blanchiment; et
800 à 1.000 millilitres d'eau déminéralisée.
immerger les pièces à plaquer dans le bain; et
déposer par électrodéposition du cuivre du bain à une température comprise entre 20°C et 30°C et à une densité de courant comprise entre 108 et 216 ampères par mètre carré (10 à 20 ampères par pied carré), en agitant sans arrêt.

7. Procédé selon la revendication 6, dans lequel l'étape d'immersion dure de 2 à 3 minutes.

8. Procédé selon la revendication 6, dans lequel l'étape d'immersion dure de 30 à 60 secondes avec application d'une tension de polarisation positive.

9. Procédé selon la revendication 6, dans lequel l'étape de préparation consiste à :
mélanger les composants du bain dans l'ordre dans lequel ils sont répertoriés dans la revendication 6, dans de l'eau déminéralisée; et
filtrer la solution du bain.
